

June 28, 1932.

C. A. PARSONS ET AL

1,865,041

CASTING OF INGOTS

Filed March 21, 1930 2 Sheets-Sheet 1



Fig. 1.



Fig. 2.

Inventors  
Charles Algernon Parsons  
and Hugh Malcolm Duncan  
By Their Attorneys  
Philip L. Rice & Kennedy

June 28, 1932.

C. A. PARSONS ET AL

1,865,041

CASTING OF INGOTS

Filed March 21, 1930 2 Sheets-Sheet 2



Fig.3.



Fig.4.

Inventors

Charles Algernon Parsons  
and Hugh Malcolm Dumeau  
By Their Attorneys

Philip Sawyer Rice Kennedy

## UNITED STATES PATENT OFFICE

CHARLES ALGERNON PARSONS AND HUGH MALCOLM DUNCAN, OF NEWCASTLE-ON-TYNE, ENGLAND; SAID DUNCAN ASSIGNEE TO SAID PARSONS; KATHARINE PARSONS, VINCENT THOMPSON, AND FREDERICK GORDON HAY BEDFORD LEGAL REPRESENTATIVES OF SAID CHARLES ALGERNON PARSONS, DECEASED

## CASTING OF INGOTS

Application filed March 21, 1930, Serial No. 437,631, and in Great Britain May 8, 1929.

This invention relates to the casting of ingots, more especially steel ingots, and is an improvement in or modification of the process described in the specification of the Patent No. 1,671,253 dated the 29th day of May, 1928.

It is an important feature of the process therein described that the surface of the molten metal should be the last to solidify and forms of burner are described for providing the necessary top-heating.

Experience in practice has, however, shown that due to the cooling influence of the side walls of the mould the solidifying of the upper portions takes place round the periphery while the centre is still fluid, with a consequent distribution of segregates that involves cutting more of the ingot to waste than is desirable.

With a view to overcoming such difficulties, the present invention consists in a process of casting steel ingots as indicated in which heat is applied in particular to the peripheral portions of the surface of the molten metal.

Referring to the accompanying diagrammatic drawings which show different forms of the invention by way of example:—

Figure 1 shows a sectional elevation of a gas-heated mould,

Figure 2 being as regards its upper half a cross-section on the line 2—2 of Figure 1 and as regards its lower half a corresponding plan;

Figure 3 shows a sectional elevation of a modified form of mould fitted with electrodes,

Figure 4 being as regards its upper half a cross-section on the line 4—4 of Figure 3 and as regards its lower half a corresponding plan.

When not otherwise indicated, the same reference symbols are used to denote corresponding parts in the different figures.

In carrying the invention into effect according to the form shown in Figures 1 and 2 and applicable to the casting of a heavy steel ingot, the mould in general is similar to that described in the specification above identified and comprises an open-topped circular body,  $\alpha$ , of heat-resisting material converging

slightly in an upward direction and strengthened by a steel casing,  $\alpha^1$ , and a removal cover,  $b$ , with apertures,  $c$ ,  $c$ , as shown. The massive chill block,  $d$ , with protecting plate,  $e$ , forms the bottom of the mould, while the molten metal is indicated at  $f$ .

According to the present invention, after preheating the mould to a high temperature of the order of molten steel and pouring the metal into the mould so preheated to leave a free surface, hot gases are introduced through the more or less tangentially disposed ducts,  $h$ ,  $h$ , so as to concentrate on the peripheral portions of the surface of the metal while heat is being continuously and simultaneously withdrawn from the molten metal by way of the base chill,  $d$ .

The hot gases thus disposed immediately above the molten surface serve both to heat the metal and also the upper part of the walls of the partly-filled mould with which latter the gases are held in contact by centrifugal force.

According to the modification of the invention shown in Figures 3 and 4, electrodes,  $i$ ,  $i$ , are inserted as shown through certain of the cover apertures,  $c$ ,  $c$ , and are directed towards the peripheral parts of the surface of the metal in the mould, immediately above which the operative arc-striking parts of the electrodes are disposed.

According to another modification of the invention, the surface of the molten metal and slag is covered with coke, coal or other combustible, jets of air, oxygen or a suitable mixture of gases being introduced laterally through the walls of the mould at the level of the coke or the like in a substantially horizontal and preferably tangential direction, as shown in Figures 1 and 2.

With any of the arrangements described above, the formation of segregates in the angle formed by the side walls and surface of the ingot by premature freezing due to cooling of the upper mould walls, is avoided or minimized, the isothermals being thus maintained more truly horizontal until solidification is complete; as a result the upper surface of the ingot is substantially plane with the segregates more closely adjacent thereto so

that a smaller quantity of metal is cut to waste.

So long as the peripheral parts of the surface are maintained fluid by heat concentrated thereon in accordance with this invention, it is found that in general the fluidity of the centre part is likewise maintained without further addition of heat, but if desired, heat may also be supplied to the centre of the surface in special cases in order to assist in securing horizontal isothermals.

The details of the processes above described may be varied without exceeding the scope of the invention.

Having now described our invention, what we claim as new and desire to secure by Letters Patent is:—

1. A process of casting metal ingots, which comprises preheating the refractory walls of an open-topped mould to a high temperature, pouring the metal into said preheated mould, withdrawing heat from said molten metal substantially wholly from the bottom thereof, and from points disposed above the free surface of said molten metal simultaneously and continuously concentrating heat directly on a narrow peripheral strip of the superficial area of said molten metal, thereby to prevent premature top freezing due to cooling of the upper mould walls and so to maintain the substantial horizontality of the isothermals throughout the cooling process.

2. A process of casting metal ingots as claimed in claim 1, in which said mould is only partly filled by said metal poured thereinto so that the mould walls project above the surface of said metal so poured and said heat is concentrated from above on a narrow peripheral strip of the superficial area of said molten metal by hot gases moving in a substantially peripheral direction and disposed directly above the surface of said molten metal, thereby simultaneously heating both the top peripheral strip of said molten metal and also heating by help of centrifugal force acting on said hot gases, the inner surface of said mould walls projecting above the surface of said molten metal.

3. A process of casting metal ingots as claimed in claim 1, in which said mould is only partly filled by said metal poured thereinto, the cross-sectional form of the mould walls immediately above said free surface of molten metal being inwardly concavely curved, and said heat is concentrated from above on a narrow peripheral annulus of the surface of said molten metal by hot gases moving tangentially to said concavely curved walls and directly above the surface of said molten metal, thereby simultaneously heating both the top peripheral strip of said molten metal and the inner surface of said concavely curved walls.

4. A process of casting metal ingots as claimed in claim 1, in which said heat is con-

centrated from above on a narrow peripheral strip of the superficial area of said molten metal by burning fuel floating on said molten metal within the area of said narrow peripheral strip.

5. A process of casting metal ingots as claimed in claim 1, in which said heat is concentrated from above on said narrow peripheral strip of the surface of the molten metal by striking electric arcs between elemental areas of said peripheral strip and the operative parts of electrodes disposed immediately thereabove.

In testimony whereof we have signed our names to this specification.

CHARLES ALGERNON PARSONS.  
HUGH MALCOLM DUNCAN.

70

75

80

85

90

95

100

105

110

110